

H. W. STOKES.  
MOLDABLE PAPER BOARD FOR CLOSURES, CONTAINERS, AND THE LIKE.  
APPLICATION FILED NOV. 14, 1917.

1,265,132.

Patented May 7, 1918.



FIG. 1.



FIG. 2.



FIG. 3.



FIG. 5.



FIG. 4.



FIG. 6.

WITNESS:

Bob. McKittrick.

INVENTOR

Henry W. Stokes  
BY  
Augustine B. Stowgley,  
ATTORNEY.

# UNITED STATES PATENT OFFICE.

HENRY W. STOKES, OF PHILADELPHIA, PENNSYLVANIA.

MOLDABLE PAPER-BOARD FOR CLOSURES, CONTAINERS, AND THE LIKE.

1,265,132.

Specification of Letters Patent.

Patented May 7, 1918.

Application filed November 14, 1917. Serial No. 202,066.

To all whom it may concern:

Be it known that I, HENRY W. STOKES, a citizen of the United States, and a resident of Philadelphia, in the county of Philadelphia and State of Pennsylvania, have invented a certain new and useful Moldable Paper-Board for Closures, Containers, and the like, of which the following is a specification.

- 10 In the manufacture of closures, containers and the like, from ordinary smooth calendered sheets of paper associated with a molding agent or compound, it is necessary or desirable to shape or bend the paper-board, consisting of the sheets and agent, into the form of the article desired, but in doing this unintentional creases and folds are formed, fine or obvious cracks are developed and there is a tendency to return to the original flat form with consequent breaking of closure or distortion of a container or other article. These defects and disadvantages are due to lack of plasticity and moldability of the paper-board, resulting from the arrangement, disposition and condition of the fibers in ordinary sheets of paper, and are present even though the ordinary sheets of paper are preliminarily finely folded, for mere folding of the sheets of paper does not improve the arrangement, disposition or condition of the fibers.

I have discovered that these serious defects and disadvantages can be avoided and a paper-board of the requisite plasticity and moldability provided by using paper fiber or pulp fabricated into crape paper in which the fibers are heaped, crisped or wrinkled into irregular heaps or ridges, so that the fibers in these mounds, heaps or ridges are so free from strain or stress as to be able to pass with ease into any other arrangement of them, by reason of the action of any pressure, stretching or other molding force, and to remain in their new association the more readily by reason of the absence of any previous strain or stress on the constituent fibers in the form in which they are first enmeshed. The molding action of the fibers, of course, takes place more readily in the presence of some moldable compound or agent which, while substantially filling the interstices of the craped, heaped or ribbed fibers, thus supporting them, offers no straining or breaking resistance to their passage into other new positions and reassessments

when the moldable compound is suitably heated or pressed, or otherwise partially or completely fluidified. A moldable and plastic paper-board made from crape paper and embodying my invention therefore contains some such compound or agent. Otherwise stated, in crape paper there are irregularly distributed areas of increased numbers of fibers, under no strain or stress, but immediately available for adaptation and re-association in connection with a moldable compound or agent and without tendency to assume their original location and form.

The invention, generally stated, is embodied in a paper board for caps, closures, containers and the like, comprising the combination of a moldable agent or compound and paper in crape form which presents the fibers in heaps, mounds or ridges and imparts plasticity and moldability to the paper-board.

In the accompanying drawings, Figure 1, is an exaggerated diagrammatic and sketchy sectional view illustrative of features of the invention.

Fig. 2, is a similar top or plan view.

Figs. 3, and 4, are views of examples of articles chosen from other articles which can be made from the composition of matter, and

Figs. 5 and 6, are extremely diagrammatic views explanatory or suggestive of a rearrangement of fibers during the molding operation of, for example, some of the parts of the articles shown in Figs. 3 and 4.

In the drawings 1, are the fibers and they are arranged in the crape paper or craped sheet fiber 2, in irregular mounds or ridges 3, which are not corrugations but are heaps, either round or linear in character, of fibers and not merely folds, although a heap on one side tends to make a valley or depression on the other, thus irregularly changing the distribution of fibers, or in other words, varying the thickness of the sheet. In the mounds or heaps the fibers may range in various directions. 4, is a moldable compound or impregnation or stiffening agent, varieties of which are well known, and of which some are moldable or plastic by heat and pressure, and some by pressure alone and of which some are water-proof and others are not. By way of further explanation examples of known moldable agents or compounds are

60

65

70

75

80

85

90

95

100

105

110

resinous admixtures of mineral fillers, resinous and waxy compounds alone and these combined with mineral fillers separately.

More than one sheet of crape paper may 5 be and usually is employed and when this is done the sheets are superposed, as shown. In what I believe to be the best embodiment of the invention, all the sheets are of crape paper, but in some cases some of them may 10 be crape paper and others of smooth paper. It is unnecessary to illustrate or particularly describe coatings which are frequently applied to the faces of the articles or sheets, because they may or may not be employed in 15 articles embodying crape paper.

When the craped sheet fiber or paper-board is molded, for example, into the forms shown in Figs. 3 or 4, or any other forms, the moldable compound separates the fibers 20 and when in a fluid state acts as a lubricant for the passage or movement and redistribution of the fibers themselves. The mounds or ridges may be described as reserve supplies of fibers for utilization in any stretching or pulling operations applied to the 25 paper-board in the production of the final products.

I have endeavored to illustrate this idea in Figs. 5 and 6, in which, Fig. 5 shows (most 30 diagrammatically) a reserve supply of fibers in the form of a heap or mound, which fibers in the molding operation may adjust themselves, as shown in Fig. 6, and in the new position of Fig. 6 there is absent from the 35 material any tendency to return to its original sheet form. In the molding operation the fibers may be straightened or they may even be heaped to a greater extent than before. The fibers may have been straightened 40 to begin with and merely readjusted through the lubricating action of the fluidified compound. The fibers are readjusted or readapted either individually or *en masse*. The ridged, mounted or craped surface of 45 the sheets provides for good adhesion with the moldable compound or agent and between the various sheets. The extent to which the paper is craped depends upon the extent of the pulling or pushing to which 50 the paper board is subjected in shaping it into the finished articles, so that if cracks or creases or a tendency to return to original form appear, as a result of any particular molding operation the heaped or ridged 55 property should be increased, and it is well understood that the amount of molding com-

pound or agent employed is variable and is well understood. The change in form from smooth to craped of the paper employed is no mere change of form or mere substitution of material but constitutes the essence of the present invention, because of the unexpected or surprising character of the results, the new mode of operation and the advance in the art. Crape paper performs the 60 function or office of presenting the fibers in a manner already described in detail, and which may be summarized by saying that the fibers are distributed by the operation involved in making crape paper not uniformly but in heaps or mounds, irregular in 65 size, shape and disposition and operative, in connection with a fluidity producing compound or agent, to readily assume and remain in new positions without rupture or 70 cracking of the sheet or web of paper-board, whereby practically perfect finished 75 articles can be produced.

In attempting to describe the arrangement of fibers in crape paper I do not desire to 80 limit the invention because the latter broadly covers the use of crape paper along with a moldable agent or compound, but my intention is to point out that there is in crape paper an arrangement of fibers which in 85 connection with a moldable or stiffening agent or compound imparts to the paper-board an unexpected property of moldability and plasticity by which it can be formed into containers, caps and various articles 90 free from cracks and capable of retaining the molded form.

What I claim is:

1. As a new article of manufacture paper-board for caps, closures, containers and the 95 like, comprising the combination of paper in crape form and a stiffening agent plastic under heat and pressure, substantially as described.

2. As a new article of manufacture paper-board for caps, closures, containers and the 100 like, comprising the combination of paper in crape form and a stiffening agent plastic under pressure, substantially as described.

3. As a new article of manufacture paper-board for caps, closures, containers and the 105 like, comprising the combination of paper in crape form and a stiffening agent consisting of a resinous admixture of mineral filler plastic under heat and pressure, substantially 110 as described.

HENRY W. STOKES.